

## Cross Reference

July 23, 1929.

P. E. EDELMAN

1,721,949

PLATING AND POLISHING ELECTRODE

Filed May 7, 1928



INVENTOR.  
Philip E. Edelman.

## UNITED STATES PATENT OFFICE.

PHILIP E. EDELMAN, OF CHICAGO, ILLINOIS.

## PLATING AND POLISHING ELECTRODE.

Application filed May 7, 1928. Serial No. 275,656.

My present invention relates to pad anodes of the class described in my copending application for U. S. Letters Patent, Serial No. 272,041, filed April 23, 1928, and has for its 5 objects (1) to include the operating chemicals in the pad itself, (2) to permit dry shipment of the pad in form operative on dipping into water, (3) to include polishing ingredients in the pad in manner operative 10 by exudation to form a mild abrasive surface for polishing, (4) to proportion the ingredients whereby the re-coating effect is greater than the abrasive or polishing effect of the electric pad, and (5) to afford inter- 15 change or renewal of operative chemical ingredients.

My electric pad affords in practice a portable practical electro-plating and polishing device in which the ingredients are proportioned for cleaning, replating, and polishing 20 a metal object without removing said object from the supporting member to which it is attached. The operations of replating the metal object and polishing same are simultaneous, with replating preponderant, so that a bright lustrous new metal coat results. This differs from mere gilding or coating by contact of solutions, pastes, or metal and solution contacts.

30 Thus where only a thin temporary coat unable to support polishing is had by gilding, solution, or solution and metal contact, my electric pad affords a homogenous hard coating simultaneously polished and able to withstand additional polishing. Also objects can be successfully coated when somewhat dirty because the abrasive action of the pad affords the necessary cleaning. Worn objects can be neatly patched and recoated 35 by this means.

40 My invention is suitable for any metal coating, as for example, nickel, cobalt, chromium, copper, silver, gold, platinum, antimony, bismuth or any suitable metallic alloys which can be electroplated. When automobile parts are to be re-finished, the car battery can be used as a source of current if the battery is grounded at its negative terminal. Or if desired, a separate battery may be used 45 or a rectifier or power unit supply source such as described in my co-pending application for U. S. Letters Patent of the United States Serial No. 192,069, filed May 17, 1927, may be employed. The voltage and current require-

ments will vary according to the metal to be 55 plated but in general my invention permits a greatly increased current density due to the simultaneous rubbing action afforded by the pad, insuring good deposits at much higher density than is customary for liquid baths. 60

My invention differs from bath dips etc. in that the electric pad is most effective when just moist and not dripping wet. There is sufficient resistance in the electrolyte formed in the pad to regulate the current flow and a 65 certain heating action is caused by the electric current flow and rubbing action of the pad which is beneficial for rapid thick deposit results.

I have discovered also that the anode metal 70 need not be the same as the metal to be plated, as in general any metal lower in the electro-motive series and substantially insoluble in the electrolyte formed in the pad is suitable. Thus for nickel plating, lead sheet affords a 75 suitable anode material, while either lead or iron is suitable for chromium plating anode material. Also, since aluminum is protected by a film formed on its surface and inasmuch as aluminum readily combines with free oxygen liberated by electrolysis, it is an advantage to use a laminated anode of sheet aluminum riveted to lead or steel by eyelet rivets. Reliance is had on the renewal of the electrolyte salts for maintaining the pad 80 operative.

Thus I prefer to use metallic salts and assisting chemicals therefor in the pad in proportion with certain readily soluble ingredients and other less soluble ingredients, as 85 exemplified in the case of nickel plating by use of powdered nickel salts consisting of a mixture in dry form of both nickel-ammonium sulphate (double salt, difficult to dissolve), and nickel sulphate (single salt, 90 readily soluble), preferably with the first named double salt in excess in the vicinity of the anode. Then when the anode pad is soaked in water a few minutes the single salt first dissolves, while the double salt serves as 95 a re-inforcing agent to maintain the electrolyte at proper plating strength.

The chemicals used depend on the metal to be plated and in general are used in more concentrated proportion in my electric pad 100 than for wet baths in tanks. I indicate by way of example, suitable chemicals but various changes and modifications may be made 105

by anyone skilled in the art within the spirit of the idea disclosed and within the scope of the appended claims.

An exemplification of the invention is had for nickel plating. The combination requires the following parts.

Reference is made to the accompanying drawing in which the figure is a diagram, partially sectioned, showing the relation of the parts.

10 A connector (A) is joined to electrode (B) formed of an aluminum and a lead sheet respectively. A wrapping pad (C) made from fabric bags surrounds electrode (B). Slowly soluble crystals reduced to powder are included by inner wrapping (C) in the vicinity of electrode (B). Soluble electrolyte chemicals are placed between the wrapping bags (C). Chemicals placed between the 15 wrappings (C) are indicated by letter (D). The chemical (D) largely is comprised by polishing powder and boric acid adjacent to the outer wrapping bag (C). A pad containing operating chemicals is thereby provided, as bags (C) are permeable to chemicals (D) which form an electrolyte about anode (B) when pad (C) is immersed or 20 wetted with water.

The combination of the figure comprises, 25 as set forth, an electric pad, or portable plating and polishing appliance.

(A.) Means to connect the anode and work to a source of electric current.

(B.) A metallic anode (which for electro-cleaning purposes may also be made a temporary cathode, when desired).

(C.) A pad, preferably containing absorbent material and a soft fabric covering, enclosing the anode and the operating chemicals.

30 (D.) Operating chemicals including metallic salts, assisting chemicals, (in substantially dry or non-spilling form), and polishing or mild abrasive powder having the property of exuding thru the outer fabric covering provided by part (C).

Thus for nickel plating and polishing, part (A) may comprise a flexible No. 14 rubber covered wire, having one end thereof soldered 35 to a battery clip attachable to the positive terminal of a storage battery, and its other end soldered or welded to the anode part (B), then protected by rubber or pitch coating so that the copper wire will not be attacked by part (D). A wire 14 feet long is suitable. Where the metal object to be coated is not grounded to the battery used for plating, a similar wire with two clips, one at each end, may be used to connect said work as a cathode 45 to said battery.

The part (B) may have an area of  $2\frac{1}{2}$  by  $3\frac{1}{2}$  inches for nickel plating and comprise a thin sheet of nickel, or sheet lead, or preferably a laminated pair of sheets, one of which 50 is aluminum and the other lead. Thin sheets

are desirable to make the electric pad flexible so that odd shapes in the work to be coated may be reached thereby. For chromium plating, the laminated electrode may be made from one sheet of lead riveted to one thin sheet of steel or aluminum. Larger or smaller anode area may be employed where desired, but the dimensions stated will suffice for passing a plating current varying from 1 to 10 amperes according to the manner in which the anode is pressed with respect to the work to be coated. Tubular rivets are suitable for holding the anode laminations together. If tin is included in the alloy to be plated, the anode materials 70 must be lower in the electromotive series than tin and insoluble in the electrolyte formed in the pad when same is dipped in water. The anode should be made with rounded corners that will not tear thru the covering material (C).

For electro-cleaning by the pad method, the described anode can be used, or preferably a duplicate anode will be used and connected as a cathode, with the work connected as the 90 anode. The electrolyte material may be, for cleaning, a mixture of water with such gritty alkali material as is used for scouring cleaners. It is desirable to have a separate cleaning electrode in order not to contaminate the 95 plating pad therewith. In use, ammonium chloride may be added to the cleaning pad. The removed coating from the work anode will then precipitate as a sludge easily washed away. Large objects can be cleaned 100 at small areas thereof without necessitating removal from attached supports, to permit recoating worn areas thereof.

The pad (C) essentially must encase the anode or electrode (B) to prevent direct 105 contact thereof with the work connected as cathode with respect thereto (or reversely, in the case of electro-cleaning). Various assemblies for the pad are suitable, an exemplification being the following combination. 110

A canvas or cotton bag is tied around the part (B). A portion of the chemicals (D) are included in this bag, and in the case of nickel plating, most of the more difficultly soluble double salts aforesaid will be included 115 in this first bag. The chemicals (D), can be loose in this bag or wrapper but may be tufted therewith by sewing or pasting tuft portions on the bag, or a piece of cellucotton or outing flannel can be used sandwiched 120 around the anode (B) to hold the chemicals (D) thereabout. Any means which will hold the chemical powders (D) with respect to electrode (B) in the bag is suitable.

A second bag or wrapper is now slipped 125 over the first bag and tied with draw strings, and may contain a further portion of the chemicals (D), but preponderant with the more soluble portions thereof. Similarly a third fabric bag or wrapping may be now 130

encased over the aforesaid second bag, with a preponderance of abrasive powder constituent of the chemicals (D).

I have found ordinary mailing bags suitable for this purpose, and this encasement by additional bags may be continued up to 6 bags if desired, though 1 or 2 or 3 bags are ordinarily all that are required. The final encasing bag should preferably be made from soft material such as outing flannel and largely contain the abrasive polishing powder and acid crystal components of the chemicals (D). The latter powders of (D) are readily able to exude or penetrate thru the pores of the last bag of pad (C) to afford effective cleansing and polishing action. Probably the multiple bags of the pad (C) afford a certain electrical diaphragm action and exert a beneficial electrical endosmosis effect. I have observed that by such construction, dirt and deposits accumulating on the outer bag in use, do not penetrate to the inner bag. The outer bag can accordingly be removed and renewed without detriment to the action after prolonged use of pad (C).

The various parts used are well known and understood but a new and useful result is afforded by the new combination thereof whereby the new result stated is attained in simple and practical manner. The polishing effect of chemicals in the outer bag is proportioned so that the plating effect simultaneous therewith is preponderant thereover.

Where desired, the bags and absorbent material (such as cellucotton) aforesaid may be sewed or fastened together, but in practice, equally good results are obtained by merely wrapping or encasing one of said coverings forming said pad (C) around the next preceding one.

The operating chemicals (D) will vary according to the work and as an example, suitable ingredients are specified for nickel plating. In general the operating chemicals (D) will include metallic salts of varying solubilities with the least soluble metallic salts nearest to the anode, also the abrasive or polishing ingredients will be preferably included only in the outer pad wrapping or bag, separately, or with the acid crystal content of chemicals (D). The abrasive or polishing material of (D) must not be capable of reacting unfavorably with the other chemicals used. I have found ordinary infusorial earth powder (tripoli) suitable. Also the preparation sold as "siliceous cleansing" powder works well. Whiting appears less suitable, and alkali cleaners cause dark streaks on the work. Pumice powder is rather too abrasive for most work but may be used with the infusorial earth if desired.

As aforesaid, the pad (C) will thus have preferably a series of fabric layers each including certain portions of the chemicals (D), though nearly as good results can be

had by a single mix of said chemicals when only two bags or coverings (C) for electrode (B) are used.

For nickel plating, suitable dry proportions are, for example—

| Chemicals                                   | Parts | 70 |
|---------------------------------------------|-------|----|
| Nickel sulphate, single salts.....          | 3     |    |
| Nickel ammonium sulphate, double salts..... | 8     |    |
| Magnesium sulphate.....                     | 1/2   |    |
| Ammonium chloride.....                      | 1     | 75 |
| Boric acid.....                             | 2     |    |
| Infusorial earth.....                       | 2     |    |

When a hard nickel is desired, cobalt sulphate or cobalt-ammonium sulphate may be substituted for the nickel sulphate single salts. Any suitable mild abrasive polish powder can be substituted for the infusorial earth. The magnesium sulphate and the ammonium chloride content may be minimized or varied as may be desired, but an excess of boric acid or some equivalent acid crystal ingredient is desirable.

The ingredients of the example are reduced to powder and intermixed as a single mixture or preferably with various proportions of the total. Thus in the latter case, 7 parts of the nickel ammonium sulphate, 1/2 part magnesium sulphate, 1/2 part ammonium chloride may be mixed and included in the first wrapping of (C) around anode (B), while the remainder may be mixed separately and included in the outer bag of pad (C). Or if a plurality of bags are used for pad (C), the outer bag may include only portions of the boric acid and all of the infusorial earth or equivalent specified. When cobalt addition is used as aforesaid precautions should be taken against the poisonous property thereof, it being desirable for the operator to wear rubber gloves or employ a wooden stick in manipulation of pad (C). The specified ingredients are not harmful to the hands of a normal person and if accidentally spilled may be washed away from other parts than the work treated, without harm. The ingredients are more or less soluble, as stated except the infusorial earth, which however is finely divided and able to exude or penetrate thru the outer bag and exert its abrasive or polishing action on the work.

In use, the pad (C) with prepared chemical content (D) is in dry or substantially dry form. It is rendered operative by brief immersion in a small jar of hot water. Excess water is rinsed therefrom and the pad (C) with operating chemicals and water content is to be used in moist condition without excess dripping water or electrolyte. After initial use, the pad (C) aforesaid may be further dipped in moistening water as stated.

The work to be refinished should be preferably first cleaned and dried, though work which is not too dirty can be refinished directly without preparation. For cleaning,

130

80

85

90

95

100

105

110

115

120

125

130

the work should be scoured or electro-cleaned, using an electric pad of the kind set forth connected as a cathode with the work connected as an anode, employing an alkali 5 scouring agent with water as the cleaning electrolyte. The work when cleaned is washed and preferably dried.

In applying the electric pad, a firm continuous motion is desirable. The pad should 10 not be left in one position on the work, but should be rubbed thereon with continuous motion. This prevents formation of spots. If spots occur by forgetting to rub as stated, they can ordinarily be removed by simply 15 further rubbing the plating pad thereover. After prolonged use the outer bag should be renewed as aforesaid.

The rubbing operation both plates and polishes the work and the result is continu- 20 ously visible. Sharp corners or depressions on the work which require building up are easily reached and patched with smooth lustrous re-finish. The plating is rapid and requires but a few minutes for a serviceable 25 durable coating. Parts worn brassy or down to copper base are easily renewed in this manner. The present invention differs from my aforesaid copending application for Letters Patent in the improvements stated and 30 especially in that the electric pad may be shipped dry ready for use, without requiring cans of operating ingredients. Also the combination specified puts the polishing ingre- 35 dient inside the last wrapping of pad (C) where it is surprisingly effective by the stated action. Readings of a series connected am- 40 meter on a 6 volt battery on average work show a current consumption averaging 5 am- peres. The deposit obtained is firm and ad-hering and does not rub off, nor crack. It 45 will even stand considerable scouring without signs of wearing thru to the base object.

I have now fully set forth an exemplification of my invention and it will be understood 45 that any metal or alloy can be plated and polished by use of suitable ingredients in chemicals (D). The various chemicals suitable for most metals and alloys are well known and understood and reference is made to "Electro-Deposition of Metals" by Lang- 50 bein-Brannt published 1924 by Henry Carey Baird & Co. New York for principles and formulas applicable to other metals. How- 55 ever in the case of chromium, I will now specify an operable mixture for (D).

For chromium plating, the work should first be cleaned and dried thoroughly and preferably coated with nickel. This may be done as herein specified or by any suitable 60 method. The nickelled surface should be cleaned, washed, and dried immediately prior to application of the chromium surface.

It seems to be an advantage to have the work warmed, as can be accomplished by 65 application of an ordinary electric heating

pad thereto just prior to application of the chromium coating.

The operator must apply the chromium plating pad quickly and smoothly with rapid motion and even pressure, to obtain lustrous result. If the pad is left on the work without rubbing, dark deposits probably containing chromates are obtained. A good coating of chromium can be had in about one minute by proper manipulation of the moistened pad. Rubber gloves should be worn, owing to the poisonous character of the chromium chemicals, and the outer pad will require frequent renewals. The results obtainable however justify the effort required, as it is not necessary to remove the metal object for repeated tank treatments as in the prior art.

The chemicals (D) used for chromium plating may be proportioned as follows:

| Chemicals                           | Parts           |
|-------------------------------------|-----------------|
| Chromic acid (readily soluble)..... | 33              |
| Chromic sulphate.....               | 1 $\frac{1}{4}$ |
| Nickel carbonate.....               | 1 $\frac{1}{4}$ |
| Infusorial earth.....               | 8               |
|                                     | 90              |

The pad (C) may be prepared with said chemicals in same manner as specified for nickelelling.

In this specification the word "parts" descriptive of proportions in chemical formulæ means "parts by weight."

The electric chromium pad should be redipped in the jar of hot water provided, as much of the chromic acid becomes dissolved therein in use. After the work is ready and preferably warmed as aforesaid, the connected electric pad is promptly and rapidly rubbed over the work portions to be coated or recoated. A vigorous motion with heavy current density will afford a bright lustrous coating of permanent character. Any chemical spilled by accident should be promptly washed away with a sponge full of warm water. It is recommended that a rubber coated fabric shield be placed around metal objects to be treated with chromium. A dexterous manipulation essentially as specified is required for satisfactory results. As aforesaid, laminated sheet lead and steel or lead sheet with aluminum is a suitable material for anode (B) for chromium application.

In any case of application of this invention, the completed work should be washed with a sponge dipped in warm water and promptly dried. Flannel cloths of outing flannel material are suitable for drying, and vigorous rubbing of finished work will bring out a lustrous appearance in a few minutes. The washing is desirable to remove traces of chemicals left on the work during the treatment. In the case of chromium plating, the washing should be done promptly after treat-

70

75

80

85

90

95

100

105

110

115

120

125

130

ment and repeated until all traces of chromium chemicals are washed away from the plated surface.

My invention permits heavy current density and localized application of the electric current, while the abrasive polish ingredient keeps the work in nascently receptive clean condition to receive the coating.

If by mistake, the operator permits the pad to remain at rest on the work so that a spotty deposit results, this can be corrected by rubbing over the spotty portions, or by re-cleaning and re-treating as aforesaid. On certain dirty work, results are facilitated by dipping the electric pad in pulverulent aluminum powder, as aluminum has great affinity for electrolytically released oxygen. For treating certain metals with chromium, I prefer to intermix aluminum powder in pulverulent form with the abrasive polishing agent employed, and sprinkle said mixture on the moistened pad. By including a small portion of tin chloride, potassium bitartrate and tartaric acid, (less than 5% of the chemical content of the electric pad), I have been able to re-finish directly over automobile bumper trim portions which showed iron rust spots prior to refinishing treatment.

It may be remarked that the combination provided affords superior results and that the crystals held in proximity to the anode maintain the electric pad in operative condition for a long time, the electrolyte formed in the moistening water tending to reach a uniform strength promptly controlled by the solubilities of the chemicals.

Difficulties met with in tank treatments in which unequal deposits are thrown on the work are avoided by the present invention as the operator can build up deposits exactly where wanted and at sharp depressions or corners on the metal object where bath deposits often fail. A minimum amount of electrolyte is handled in the pad and all the current used is effective in the electro-plating, and assisting heating effect caused by the current passing thru the resistance afforded

by the moistened pad. Even the poisonous chromium electrolyte is thereby handled in such restricted amount that fume dangers are largely avoided by this means.

In the case of metal hardware or other parts not already connected to the negative pole of a storage battery, the operator uses the clipped wire to connect same thereto and finishes the operations as set forth, moving the negative clip to different portions of the work under treatment so as to permit the entire surface to be coated to be treated. The flexible nature of the pad (C) permits odd shapes of articles to be reached, and in general it will be observed that the ratio of active anode surface to the portion of the work temporarily connected as cathode is equal to or greater than unity, whereby the desirable oxidation-reduction potential effects at the anode and cathode are correctly maintained.

The general appearance of the electric pad and a suitable mode of use has already been described in my aforesaid copending patent application. The improvements of the present invention have been particularly pointed out. Various changes and modifications are permissible within the scope of the appended claims.

I claim:

1. A plating and polishing anode having a fabric cover therefor, concentrated chemicals in substantially solid form held within said fabric cover, and a finely divided polishing powder combined with said chemicals and proportioned to penetrate therethrough when said fabric cover is wetted with water.

2. An electroplating and polishing device consisting of an electrode, a mixture of electrolyte forming chemicals and polishing powder held wrapped thereabout, a wrapper for said chemicals and polishing powder, and means to attach said electrode to a source of electric current.

In witness whereof I have hereunto set my hand this 4th day of May, 1928.

PHILIP E. EDELMAN.